

## UNITED STATES PATENT OFFICE.

VICTOR VILLIGER AND HEINRICH VON KRANNICHFELDT, OF LUDWIGSHAFEN-ON-THE-RHINE, GERMANY, ASSIGNEES TO BADISCHE ANILIN- & SODA-FABRIK, OF LUDWIGSHAFEN-ON-THE-RHINE, GERMANY, A CORPORATION OF GERMANY.

## FAST DYEING.

No Drawing.

Application filed July 9, 1920. Serial No. 395,075.

*To all whom it may concern:*

Be it known that we, VICTOR VILLIGER and HEINRICH VON KRANNICHFELDT, citizens of the Swiss Republic, residing at Ludwigshafen-on-the-Rhine, Germany, have invented new and useful Improvements in Fast Dyeing (for which we have filed an application in Germany April 28, 1917), of which the following is a specification.

10 Our invention relates to methods of dyeing and printing with certain coloring matters.

In the specification of the co-pending application, Serial No. 395,182, a green condensation product is described which can be obtained from alpha-napthoquinone for example by suitably heating in the presence of water.

We have now found that by means of the 20 said green product excellent fast shades can be produced on both vegetable and animal fibers. The dyeing can be effected from the yellow vat of the green product, or by the padding or printing methods used with vat dyestuffs. Fiber which has been thus incorporated with the aforementioned green coloring matter can be recognized by the following reactions:

Upon spotting with dilute caustic soda lye 30 of say 10 per cent the green color turns brown, but on washing with water the original color comes back; upon treatment with nitric acid it changes to a yellow color; when spotted with other dilute acids or with a 35 hydrochloric acid solution of stannous chlorid, however, it remains practically unchanged.

The following examples illustrate this invention and the manner of carrying the 40 same into practical effect, but the invention is not limited thereto:

*Examples for dyeing.**1. For 20 kilos of wool.*

45 One kilogram of the green condensation product, which has preferably been brought into a fine state of division in the usual man-

ner, is added to the dyebath (temperature 60 degrees to 65 degrees centigrade) of 1000 50 litres of water containing a little anhydrous sodium hydrosulfite added in the form of powder. One and a half litres of 30 degrees Baumé caustic soda and 3 kilos of anhydrous sodium hydrosulfite (in powder) 55 are next added and well stirred in. An addition of 10 kilos of calcined Glauber's salt causes the vat to draw more rapidly.

After working the whole in the bath for about 1½ hours at about 65 degrees centigrade 60 it is lifted, squeezed in the usual way, oxidized in the air, and then rinsed.

Ammonia or sodium carbonate may be used in place of caustic soda.

*2. For 22.5 kilos of cotton yarn.*

65 Six and three quarters kilos of a 10 per cent paste of the green condensation product are passed through a sieve into 1000 litres of water at ordinary temperature, 3 litres of 70 30 degrees Baumé caustic soda and 2 kilos of anhydrous sodium hydrosulfite (powder) being added and well stirred. When the vat is quite ready for use, the wetted and centrifuged yarn is placed therein and worked 75 for about an hour. After the yarn has been lifted, it is developed in the air, well rinsed, and finished off in the usual way. The bath does not become completely exhausted; but this result may be attained by adding about 80 20 kilos of calcined Glauber's salt.

*3. For 45 kilos of cotton yarn.*

2.25 kilos green condensation product (10 85 per cent paste),  
4.50 kilos sodium sulfid crystals,  
3-4½ kilos calcined soda

are dissolved by suffusion with boiling water, assisted by stirring. This solution is added 90 to the boiling dyebath—the volume of which should be as small as possible—and 4.5 kilos of calcined Glauber's salt (common salt or industrial salt) are stirred in. After thoroughly stirring, the yarn is dyed in the boiling bath for an hour, being afterwards fin-

ished off in the manner usual in the case of sulfur dyes.

*Examples for padding. 1.*

- 5 100 grams green condensation product (10 per cent paste).  
 150 grams gum thickening 1.1.  
 750 cc. water.  
 10 1000 grams.

The fabric is padded with the mixture and dried.

Development is effected on the jigger, in a 15 bath of—

- 0.5 litre 40 degrees Baumé caustic soda.  
 300 grams anhydrous sodium (powder) hydrosulfite.  
 20 2.5 kilos calcined Glauber's salt.  
 100 litres water at 50 degrees to 60 degrees centigrade.

The goods are then rinsed, slightly acidified, rinsed again and soaped.

25 A white discharge can be produced on the padded fabric by means of Rongalite CL, just as with vat-dyed fabrics.

2.

- 30 30 grams green condensation product (10 per cent paste).  
 125 grams gum thickening 1.1.  
 25 grams ferrous sulfate.  
 35 3 grams tin salt.  
 10 grams 50 per cent lactic acid.  
 807 cc. water.  
 1000 grams.

40 The fabric is padded with the mixture, dried in the hot flue, developed on the wide-open washing machine, in a bath of 100 litres of 10 degrees Baumé caustic soda and 15 kilos of Glauber's salt for about  $\frac{1}{2}$  a minute, 45 given a short rinsing at 75 degrees centigrade acidified in 3 degrees Baumé sulfuric acid, rinsed again and soaped.

*Examples for printing. 1.*

- 50 150 grams green condensation product (10 per cent paste).  
 90 grams ferrous sulfate.  
 15 grams tin salt.  
 55 25-50 grams tartaric acid.  
 720-695 grams British-gum thickening 1.1.  
 1000 grams.

When printed, the fabric is dried, and then 60 placed in a bath 19-20 degrees Baumé caustic soda at 75 degrees centigrade for about 20-30 seconds, rinsed, neutralized in 3 degrees Baumé sulfuric acid, rinsed and soaped.

2. 65  
 150 grams green condensation product (10 per cent paste).  
 60 grams stannous oxid paste (50 per cent).  
 50 grams glycerine.

70  
 740 grams thickening T.  
 1000 grams.

*Thickening T.*

- 75  
 300 grams dextrin thickening 1200:800.  
 340 grams gum thickening 1.1.  
 1000 grams caustic soda (45 degrees Baumé).  
 60 grams oil of turpentine.

80 After printing, the fabric is dried at 40 degrees to 45 degrees centigrade, then fixed for 5 minutes in a rapid steamer (air being excluded), washed and soaped.

3.

- 85  
 150 grams green condensation product (10 per cent paste).  
 100 grams glycerine.  
 150 grams carbonate of potash.  
 60 grams Rongalite C. dissolved in  
 50 grams water.  
 490 grams British gum thickening 1.1.

1000 grams.

95  
 The goods when printed are dried, then fixed for 5 minutes in the rapid steamer (air being excluded) washed, soured, washed again and soaped.

*Colored discharge printing.*

The fabric previously dyed—as usual—with dischargeable substantive dyestuffs, is printed with—

- 105  
 200 grams green condensation product (10 per cent paste).  
 100 grams glycerine.  
 150 grams carbonate of potash.  
 100 grams Rongalite C.  
 450 grams British gum thickening 1.1.

110  
 1000 grams.

115  
 After printing, it is dried, fixed for about 5 minutes in the rapid steamer, with exclusion of air, washed, soured and soaped.

Now what we claim is—

120  
 1. The process of producing green dyeings on textile fiber by treating it with a green condensation product of alpha naphthoquinone, insoluble in water, in the presence of a reducing agent and oxidizing the reduction product on the fiber so treated.

125  
 2. The process of producing green dyeings on textile fiber by treating it with a green condensation product of alpha naphthoquinone, insoluble in water, after transforming it into a soluble leuco-compound by

means of hydrosulfite and alkali, and oxidizing the leuco-compound on the fiber.

3. As a new article of manufacture a green textile fiber formed by treating the fiber 5 with a green condensation product of alpha naphthoquinone, insoluble in water, in the presence of a reducing agent, and oxidizing the fiber after the treatment, the characteristics of which are that when treated 10 with caustic soda solution it turns brown, this color re-turning to green upon subse-

quent washing with water and that upon treatment with nitric acid it shows a yellow color and that the fiber when spotted with dilute acids or with a hydrochloric acid solution of stannous chlorid remains practically unchanged. 15

In testimony whereof we have hereunto set our hands.

VICTOR VILLIGER.

HEINRICH VON KRANNICHELD.